

# UNITED STATES PATENT OFFICE.

SOPHIE E. STEVENSON, OF CHICAGO, ILLINOIS.

## COMPOUND.

No. 836,223.

Specification of Letters Patent.

Patented Nov. 20, 1906.

Application filed March 11, 1905. Serial No. 249,532.

*To all whom it may concern:*

Be it known that I, SOPHIE E. STEVENSON, a citizen of the United States, residing at Chicago, in the county of Cook and State of Illinois, have invented certain new and useful Improvements in Compounds; and I do hereby declare the following to be a full, clear, and exact description of the invention, such as will enable others skilled in the art to which it appertains to make and use the same.

The nature of this invention consists in producing a compound which when hot is plastic, but which when cold is hard, yet sufficiently elastic to prevent cracking in low temperature and still retain its firmness in warm weather.

Another feature is to produce a compound which will be practically indestructible by the elements—heat, cold, rain, snow, ice, or atmosphere.

Another object is to produce a compound which may be readily repaired without having to remove the previous coating.

Another object is to produce a compound which will not ignite or burn under any ordinary circumstances, such as the burning of adjacent buildings or the dropping of sparks or fire thereon.

Another object is to produce a compound which when warm is plastic and may be

formed in various shapes for building purposes and elsewhere—such as shingles, thin boards, eaves-troughs, ornaments, &c.—which may be applied and fastened by nails, 35 if desired.

These objects are attained by the admixture of substantially equal parts constituting proper proportions of Portland cement, heated asphaltum, pulverized or ground common brick or burnt clay bound together by any suitable fibrous material, such as asbestos fiber or mineral wool, the object of the latter ingredient being to bind the other parts when molded in thin slabs or in other 40 forms, so that nails, screws, or other hard substances may be driven through when the mass is cold without cracking the composition.

I claim as new—

A compound consisting of substantially equal parts of cement, asphaltum, ground or pulverized common brick or burnt clay, the entire mass being mixed and bound together by a fibrous material. 50

In testimony whereof I affix my signature in presence of two witnesses.

SOPHIE E. STEVENSON.

Witnesses:

GEORGE F. LUST,  
M. NORBORG.